

May 6, 1958

C. A. STRATTON  
ORGANOPHILIC BENTONITE BODIED LUBRICANT  
CONTAINING A NITROPARAFFIN

Filed Sept. 2, 1954

2,833,720



BY C. A. Stratton  
Hudson and Young  
ATTORNEYS

1

2,833,720

**ORGANOPHILIC BENTONITE BODIED LUBRICANT CONTAINING A NITROPARAFFIN**

Charles A. Stratton, Caney, Kans., assignor to Phillips Petroleum Company, a corporation of Delaware

Application September 2, 1954, Serial No. 453,721

18 Claims. (Cl. 252—49.7)

This invention relates to lubricants. In one of its more specific aspects, this invention relates to bodied lubricants. In another of its more specific aspects, this invention relates to lubricants bodied by a dispersion of organophilic bentonite in a lubricating liquid. In another of its more specific aspects, it relates to a method for bodying lubricants.

This application is a continuation-in-part of my application, Serial No. 342,759, filed March 16, 1953, now abandoned.

In the production of bodied lubricants, it is customary to prepare solutions or dispersions of soaps in lubricating oils, the function of the soaps being to body up the oils to grease consistency. Soaps commonly used for this purpose are the metal salts of long carbon chain saturated and unsaturated fatty acids as, for example, potassium oleate, magnesium stearate, aluminum palmitate, etc., although salts of aromatic-acids, such as lead naphthenate, are also useful. It is commonly observed that lubricants consisting of these soap-in-oil dispersions have a relatively high thermal coefficient of viscosity and that at temperatures often encountered in machinery under normal operating conditions these greases become fluid, resulting in loss of the lubricant and damage to the machinery. This is to a considerable extent a function of the melting point of the soap. Thus, the magnesium, zinc, or aluminum soaps would not be desirable for high temperature applications because of their low melting points. The alkali soaps, while possessing higher melting points, up to 175° C., are subject to hydrolysis by moisture, which gives rise to deleterious alkalinity, and are, therefore, not entirely suited to some conditions of use. Other additives, such as clay and asphaltic materials, are sometimes used to increase the load bearing capacity and the high temperature viscosity of greases; the clays, however, introduce abrasive material, and the organic bodying agents increase the low temperature consistency to such a degree that starting of cold machinery is difficult.

One more recently developed type of bodied lubricant is one formed by colloidally dispersing an organophilic clay, commonly called bentone, in an organic lubricating liquid, such as a petroleum lubricating oil, a synthetic lubricating oil, such as a diester or heavier polyester, or a mixture of such lubricating oils, in a manner to obtain a gel or "grease." The clays which are useful as starting material for making the modified clay in accordance with this invention are those exhibiting substantial base-exchange properties, and particularly those exhibiting comparatively high base-exchange properties and containing cations capable of more or less easy replacement. The clays particularly contemplated herein include the montmorillonites, viz., sodium, potassium,

2

lithium, and other bentonites, particularly of the Wyoming types; magnesium bentonite (sometimes called hectorite) and saponite; also nontromite and attapulgite, particularly that of the Georgia-Florida type. These clays characterized by an unbalanced crystal lattice, are believed to have negative charges which are normally neutralized by inorganic cations. As found in nature, therefore, they exist as salts of the weak clay-acid with bases, such as the alkali- or alkaline-earth metal hydroxides. 5 Bentonites which are particularly useful are the swelling bentonites of the Wyoming type and the swelling magnesium bentonites of the hectorite type.

An organophilic bentonite, commonly used in the manufacture of bodied lubricants from mineral lubricating oils, is formed by replacing the exchangeable inorganic cations of the bentonite with organic cations from salts of aliphatic, cyclic, aromatic and heterocyclic amines, primary, secondary and tertiary amines and polyamines, and quaternary ammonium compounds, such as 10 dimethyldicetyl-ammonium hydroxide. The bentonite is first hydrated in a very dilute dispersion to separate the unit particles and is then purified by super-centrifuging to achieve complete removal of non-clay impurities which would impart an abrasive character to the finished lubricant. 15 The reactive exchangeable inorganic cation, such as sodium or potassium, of the dispersed bentonite is replaced by the addition of the salt referred to above and the modified clay is then filtered, washed, dried and ground into a fine powder. Increasing the chain length 20 of an alkyl ammonium cation used to replace the exchangeable inorganic cation increases the organophilic properties of the modified bentonite. A more complete disclosure of the preparation of organophilic bentonite will be found in United States Patent 2,531,427, 25 issued to E. A. Hauser.

The following are objects of this invention.

An object of this invention is to provide an improved lubricant. Another object of this invention is to provide an improved bodied lubricant. Another object of 40 the invention is to provide an improved lubricant bodied by an organophilic clay. Another object of the invention is to provide a lubricant bodied by dispersing an organophilic clay in an organic lubricating liquid with acetone and a nitroparaffin having from 1 to 3 carbon atoms. Another object of the invention is to provide a method for producing an improved bodied lubricant. Other and further objects of this invention will be apparent upon study of the accompanying disclosure.

Broadly speaking, this invention comprises the bodying 45 of an organic lubricating liquid with an organophilic bentonite clay in the presence of a nitroparaffin having from 1 to 3 carbon atoms per molecule. The use of such nitroparaffins as dispersion agents results in a grease which has good consistency. However, I have discovered that over and beyond that improvement, the formation 50 of a gel which has not only good consistency but also good work stability by dispersion of an organophilic bentonite in an organic lubricating liquid is aided by the addition of a small amount of acetone together with a nitroparaffin selected from the group of nitromethane, nitroethane, 2-nitropropane and 1-nitropropane. The adaptability of the 2-nitropropane and 1-nitropropane as a portion of the dispersion agent is dependent upon 55 whether or not the grease which is desired is a relatively soft grease. Furthermore, as will be disclosed hereinafter, a greater amount of each of the nitroparaffins is necessary to obtain a minimum unworked micropene-

tration than is necessary when using nitromethane or nitroethane.

Dispersion agents, such as ethyl acetate, acetic acid, acetone, methyl alcohol, ethyl alcohol, benzoyl chloride, butyl stearate, coconut oil, cyclohexanone, ethylene dichloride, ethyl ester, furfural, isoamyl acetate, methyl ethyl ketone, and nitrobenzene, have been disclosed by the prior art as being solvating agents which can be used in creating an organophilic bentonite clay thickened grease composition. I have found that the dispersion of an organophilic bentonite in a lubricating liquid to form a gel having good consistency and also good work stability can be facilitated by the use of a combination of acetone and at least one of the nitroparaffins of the group of nitromethane, nitroethane, 2-nitropropane and 1-nitropropane. The prior art has not suggested the use of such materials as dispersing agents in the formation of an organophilic bentonite clay thickened grease composition nor has it suggested the use of combinations of nitroparaffins and acetone to provide an organophilic bentonite clay thickened grease composition having improved work stability characteristics. I have discovered that the suitability of the alkyl nitro-paraffins is inverse to the number of carbon atoms in the alkyl radical. Of the two nitrop propane, 2-nitropropane is much more adaptable for use as a dispersion agent than is 1-nitropropane, either alone, in combination with another nitroparaffin or in combination with acetone.

Better understanding of this invention will be obtained upon reference to the drawing which is a graph showing a comparison of the effect on grease consistency of the dispersant properties of the materials used in this invention as contrasted with certain dispersants from the prior art.

The amount of dispersing agent which is utilized in my grease is dependent upon not only the specific dispersing agent, but is also dependent upon the concentration of the organophilic bentonite clay, the type of that clay, such as "Bentone 18," "Bentone 34," etc., and the specific lubricating liquid used. In general, the organophilic bentonite clay is used in a concentration within the range of from 2 to 35 percent, depending upon the specific grade of grease desired. The amount of dispersing agent which is used varies above 0.25 weight percent, generally within the range of from 0.25 to 6 percent by weight, the specific amount once again being dependent upon the bentonite concentration, the type of organophilic bentonite clay used and the lubricating liquid used. I have discovered that the alkyl nitroparaffins having from 1 to 3 carbon atoms per molecule can be used in the above concentrations. If desired, they can be used in combination. I have further discovered that nitroparaffins having from 1 to 3 carbon atoms per molecule, and particularly nitromethane or nitroethane, can be utilized in admixture with acetone which is a conventional dispersion agent for an organophilic bentonite clay, so as to obtain a grease which has a better consistency than does a grease which is formed utilizing acetone in an amount equal to the total amount of the mixture of acetone and nitroparaffin. I have found that an improved organophilic bentonite clay type grease can be formed when using at least 0.25 percent by weight total dispersant. When a mixture of acetone and a nitroparaffin is used as the dispersant in amounts within the range set forth above, the grease is improved when the nitroparaffin, preferably nitromethane or nitroethane, is present in an amount of at least 0.05 percent by weight.

The bodied lubricant is formed from an organic lubricating liquid, such as petroleum mineral oil, polyesters, silicone oils, and the like; when using one or more of these alkyl nitroparaffins alone or in combination with acetone as a dispersion agent. Outstanding properties of bodied lubricants formed with organophilic bentonite clay, such as consistency in temperature characteristics, and the like,

are improved by the use of at least one of the alkyl nitroparaffins as a part of the dispersion agent.

The preparation of a bodied lubricant from an organophilic bentonite clay in a lubricating liquid is a rather simple operation which is accomplished by thoroughly mixing the lubricating liquid and the organophilic bentonite clay with a dispersion agent. In some instances, it is advantageous to heat the mixture or work the mixture in a milling operation. However, such steps are not always necessary.

In the preparation of a grease of the instant invention, it is preferred to use a lubricating oil, such as a mineral lubricating oil, a polyester oil, or a silicone fluid, which is oxidant resistant. The selection of the specific type of oil for use in this grease depends to a large extent upon the temperatures at which it is to be used. Oils which contain aromatics, as shown by low viscosity indices, produce greases which give higher consistencies at lower temperatures than do oils of lesser aromatic content with higher viscosity indices. When greases are to be used at high temperatures, however, high viscosity oils are preferably utilized for the reason that less heat breakdown is encountered with the use of such oils. Polyester oils and silicone fluids are particularly useful in the production of greases to be used at high temperatures, as such oils are particularly heat-resistant.

The dispersion of organophilic bentonite clay in the oil phase may be accomplished rather easily while using a cold oil. The dispersion can be made even more readily, however, by heating the oil to a temperature below its decomposition point but preferably to a temperature but slightly above atmospheric temperature.

Minor proportions of conventional oxidation inhibitors, such as mercaptoaryl thiazoles, aminophenols, phenylene diamines, and phenyl- $\alpha$ -naphthyl amine, may be incorporated in the grease for the purpose of improving the oxidation resistance of the oil base.

The percentage of organophilic bentonite clay which may be used to produce a satisfactory lubricant of this invention usually lies in the range of 2 to 35 weight percent based on the finished lubricant. I prefer to use clay loading in the range of 3 to 15 weight percent of the finished product lubricant, since such loadings result in excellent bodied lubricants and it is economically desirable to use as low clay loadings as possible to obtain the desired bodying.

Better understanding of this invention will be obtained upon reference to the following specific examples which are meant to be exemplary and not to be unduly limiting of the invention.

#### EXAMPLE I

Bodied lubricants of similar compositions were prepared from several different petroleum mineral oil stocks and including minor proportions of acetone or nitromethane. Given quantities of commercial grade dimethyl dicetyl ammonium bentonite (Bentone 34), an organophilic bentonite clay available from the National Lead Company, were mixed with small quantities of selected petroleum mineral oil lubricating blending stock to form a slurry and minor amounts of acetone or nitromethane were added to selected mixtures. Additional lubricating blending stock was then added at room temperature to form a bodied lubricant. After thorough mixing, the admixture was milled in a Navy grease worker using a worker plate containing 0.06 inch holes for 1000 strokes. The bodied lubricant was then de-aerated for ten minutes under a mechanical vacuum to remove the entrained air bubbles. These lubricants were then tested with a penetrometer, as described in ASTM Test D-217-44T, but modified so as to use a micropenetrometer needle, plunger and cup as described by Kaufman, Finn, and Harrington in "Industrial and Engineering Chemistry," Analytical Edition 11, 108-110 (1939). The lubricant composition and micropenetrations are set forth below in Table I.

5  
Table I

|                                    |       |       |
|------------------------------------|-------|-------|
| "Bentone 34"                       | 7.0   | 7.0   |
| 20 Lubricating oil blending stock  | 91.5  | 91.5  |
| Nitromethane                       | 1.5   |       |
| Acetone                            | 1.5   |       |
|                                    | 100.0 | 100.0 |
|                                    | 105   | 84    |
| "Bentone 34"                       | 5.0   | 5.0   |
| 250 Lubricating Oil blending stock | 93.5  | 93.5  |
| Nitromethane                       | 1.5   |       |
| Acetone                            | 1.5   |       |
|                                    | 100.0 | 100.0 |
|                                    | 193   | 183   |
| "Bentone 34"                       | 7.0   | 7.0   |
| 200 Lubricating oil blending stock | 91.5  | 91.5  |
| Nitromethane                       | 1.5   |       |
| Acetone                            | 1.5   |       |
|                                    | 100.0 | 100.0 |
|                                    | 382   | 319   |

As shown by the penetration tests, the bodied lubricants prepared with nitromethane as the dispersant, have greater consistency than the bodied lubricants of similar composition prepared with acetone as the additive material.

#### EXAMPLE II

5.25 grams of "Bentone 34" were slurried into 25.0 grams of 20 lubricating oil blending stock. 1.12 grams of ethyl acetate were added, and the mixture was stirred until a gel was obtained. The gel was weak, having a micropenetration, obtained as disclosed in Example I, of 356. The "Bentone" content of this grease was higher than is commercially feasible, and when additional oil was added to the grease to bring the "Bentone" content down to a reasonable value, the gel broke up completely.

#### EXAMPLE III

Two greases were prepared by stirring "Bentone 34" into a 20 lubricating oil blending stock until a smooth

5 mometer suspended in the sample. Each sample was maintained at a temperature of 400° F. for one hour and 45 minutes. During the heating over this period, grease 2 blackened considerably more than grease 1, and it appeared that the former was undergoing more serious decomposition than the latter. However, micropenetration measurements obtained as disclosed in Example I indicated that such was not the case. The samples were cooled to room temperature, and were thoroughly stirred. The following micropenetrations were measured:

|    |                  | Grease 1 | Grease 2 |
|----|------------------|----------|----------|
| 15 | Micropenetration | 256      | 150      |

10 Therefore, as shown by these data, the grease prepared by using nitromethane as a dispersant had a better temperature resistance than the one using acetone as the dispersant.

#### EXAMPLE IV

Several comparative greases were formed in the following manner. 5.2 grams of "Bentone 34" was added 25 to 92.5 grams of 20 lubricating oil blending stock. The "Bentone 34" was allowed to become wetted by the oil and settle therein. The mixture was thereafter stirred in a mixer for five minutes to effect a uniform slurry. Nitromethane was added to the slurry and the slurry 30 was thereafter mixed for a period of five minutes. Acetone was then added and the mixture was stirred for thirty minutes. The mixture was then milled in a Charlotted mill, model ND-1 with a three horse-power motor and a T-grooved rotator and stator at 0.003 inch clearance and 257 ml./min. The same procedure was utilized 35 in forming greases using only nitromethane or acetone as the dispersion agent, except that the mixtures in those cases was stirred for a total of thirty minutes to obtain thorough mixing. Work stability of the greases was determined and the results are set forth below in Table III.

Table III

|                                    |       |       |       |        |       |        |       |
|------------------------------------|-------|-------|-------|--------|-------|--------|-------|
| "Bentone 34"                       | 5.5   | 5.5   | 5.5   | 5.5    | 5.5   | 5.5    | 5.5   |
| 20 Lubricating oil blending stock  | 92.5  | 92.5  | 92.5  | 92.5   | 92.5  | 92.5   | 92.5  |
| Nitromethane                       | 2.0   | 1.5   | 1.0   | .75    | .5    | .25    |       |
| Acetone                            |       | .5    | 1.0   | 1.25   | 1.5   | 1.75   | 2.0   |
|                                    | 100.0 | 100.0 | 100.0 | 100.00 | 100.0 | 100.00 | 100.0 |
| A. S. T. M. Standard Penetrations: |       |       |       |        |       |        |       |
| 0-strokes                          | 295   | 303   | 310   | 321    | 325   | 342    | 385   |
| 60-strokes                         | 292   | 302   | 305   | 313    | 319   | 343    | 385   |
| 10,000-strokes                     | 338   | 343   | 338   | 341    | 347   | 369    | 411   |

slurry was obtained. The dispersant (acetone or nitromethane) was then stirred into the "Bentone" oil slurry, and this mixture was passed three times through a laboratory model Charlotte colloid mill at a clearance of 0.003 inch. The grease was deaerated by means of a vacuum produced by a rotary pump. The compositions of the bodied lubricants and micropenetrations are set forth below in Table II.

Table II

|                                   | Grease 1 | Grease 2 |
|-----------------------------------|----------|----------|
| 20 Lubricating oil blending stock | 732 G.   | 732 G.   |
| "Bentone 34"                      | 66       | 56       |
| Acetone                           | 12       |          |
| Nitromethane                      |          | 12       |
| Micropenetration                  | 100      | 85       |

A sample of each of these bodied lubricants was heated on a hot plate in a 50 milliliter beaker. The two samples were heated side by side on the same hot plate and the temperature of each was determined by means of a ther-

5 mometer suspended in the sample. Each sample was maintained at a temperature of 400° F. for one hour and 45 minutes. During the heating over this period, grease 2 blackened considerably more than grease 1, and it appeared that the former was undergoing more serious decomposition than the latter. However, micropenetration measurements obtained as disclosed in Example I indicated that such was not the case. The samples were cooled to room temperature, and were thoroughly stirred. The following micropenetrations were measured:

|    | Grease 1 | Grease 2 |
|----|----------|----------|
| 15 | 256      | 150      |

10 Therefore, as shown by these data, the grease prepared by using nitromethane as a dispersant had a better temperature resistance than the one using acetone as the dispersant.

20

are required to disperse 7 weight percent "Bentone 34" in 20 lubricating oil blending stock.

Various modifications of this invention will be apparent to those skilled in the art. Such modifications are believed to be within the spirit and the scope of this invention as set forth in this disclosure.

I claim:

1. A bodied lubricant comprising an organic lubricating liquid; a sufficient amount of an organophilic bentonite clay to thicken said lubricating liquid to a grease consistency; and an amount of a mono-nitroparaffin containing from 1 to 3 carbon atoms per molecule sufficient to disperse said clay.

2. The lubricant of claim 1 wherein said nitroparaffin is nitromethane.

3. The lubricant of claim 1 wherein said nitroparaffin is nitroethane.

4. The lubricant of claim 1 wherein said nitroparaffin is 2-nitropropane.

5. The lubricant of claim 1 wherein said nitroparaffin is 1-nitropropane.

6. A bodied lubricant comprising between 65 and 97 weight percent of an organic lubricating liquid; between 2 and 35 weight percent of an organophilic bentonite clay, and between 0.25 and 6 weight percent of a mono-nitroparaffin containing from 1 to 3 carbon atoms per molecule.

7. A bodied lubricant comprising between 65 and 97 weight percent of an organic lubricating liquid; between 2 and 35 weight percent of an organophilic bentonite clay, and between 0.25 and 6 weight percent of a mixture of acetone and a mono-nitroparaffin containing from 1 to 3 carbon atoms per molecule, wherein said nitroparaffin is present in said mixture in an amount of at least 0.05 percent by weight.

8. A lubricating composition having an organic lubricating liquid base bodied with an organophilic bentonite clay and containing as a dispersant 0.25 to 6 weight percent of a mixture of acetone and nitromethane wherein said nitromethane is present in an amount of at least 0.05 percent by weight.

9. A bodied lubricant comprising between 65 and 97 weight percent of an organic lubricating liquid; between 2 and 35 weight percent of an organophilic bentonite clay, and about 2 percent by weight of dispersant material consisting essentially of nitromethane in the range of from 0.3 to 0.8 percent and acetone in the range of from 1.2 to 1.7 percent by weight.

10. In producing a bodied lubricant by incorporating an organophilic bentonite clay in an organic lubricating liquid, the improvement which comprises using as at least

a portion of the dispersant, a mono-nitroparaffin containing from 1 to 3 carbon atoms per molecule.

11. A bodied lubricant comprising between 80 and 95 weight percent of an organic lubricating liquid; between 3 and 15 percent by weight of an organophilic bentonite clay; and between 0.25 and 6 weight percent of a mono-nitroparaffin containing from 1 to 3 carbon atoms per molecule.

12. A bodied lubricant obtained by dispersing between 2 and 35 weight percent of an organophilic bentonite clay in from 65 to 97 percent by weight of an organic lubricating liquid in the presence of between 0.25 and 6 weight percent of a mono-nitroparaffin containing from 1 to 3 carbon atoms per molecule.

13. A bodied lubricant consisting essentially of an organic lubricating liquid thickened to a grease consistency in the presence of a dispersing amount of a mono-nitroparaffin containing from 1 to 3 carbon atoms per molecule with between 2 and 35 percent by weight of a complex formed by reacting a bentonite clay with a salt of a material selected from the group consisting of amines and quaternary ammonium compounds.

14. The lubricant of claim 13 wherein said organic lubricating liquid is thickened in the presence of nitromethane.

15. The lubricant of claim 13 wherein said organic lubricating liquid is thickened in the presence of nitroethane.

16. The lubricant of claim 13 wherein said organic lubricating liquid is thickened in the presence of 2-nitropropane.

17. The lubricant of claim 13 wherein said organic lubricating liquid is thickened in the presence of 1-nitropropane.

18. A bodied lubricant comprising between 65 and 95 weight percent of an organic lubricating liquid; and between 5 and 35 weight percent of an organophilic bentonite, thickened to grease consistency in the presence of between 0.4 and 5 weight percent of nitromethane.

#### References Cited in the file of this patent

#### UNITED STATES PATENTS

|           |            |              |
|-----------|------------|--------------|
| 2,662,056 | McCarthy   | Dec. 8, 1953 |
| 2,662,057 | McCarthy   | Dec. 8, 1953 |
| 2,662,058 | McCarthy   | Dec. 8, 1953 |
| 2,677,661 | O'Halloran | May 4, 1954  |

#### OTHER REFERENCES

"Organophilic Bentonites—Swelling in Organic Liquids" by John Jordan, Journal of Physical and Colloid Chem., pages 294, 305, vol. 53, No. 2, February 1949.